

## UNITED STATES PATENT OFFICE

1,951,911

MOLD FOR CASTINGS OF IRON AND  
NONFERROUS METALS

Max Heusser, Winterthur, Switzerland

No Drawing. Application December 11, 1931,  
Serial No. 580,506. In Switzerland December  
13, 1930

6 Claims. (Cl. 22—188)

It is known that the size of grain in the structure of a casting depends to a large degree on the rate of cooling and therefore on the thermal conductivity of the mold. When the heat is led away slowly from the mold, and the casting is therefore cooled slowly, the structure of the casting is open grained, whilst when cooling or heat transmission through the material of the mold is more rapid, a fine-grained structure is obtained.

5 It is not yet known to make any use of this fact, since the known methods of improving the quality of castings by adopting molds made of metal, through which the thermal conductivity at certain parts shall be changed as compared with

10 that at other parts, have the disadvantage that in consequence of the sudden variation of the thermal conductivity of the material used, great differences occur in the quantities of heat transmitted from the casting. This leads to an all too rapid chilling and consequently an undesirable hardness of the material, so that not only is annealing required in order to make the structure more uniform, but difficulties for machining are also created. The known method of coating the

15 surface of the mold with graphite cannot reduce this injurious effect, since it solely prevents the mold burning and has no influence worth mentioning on the thermal conductivity of the material of the mold.

20 The purpose of this invention is to control the rate of cooling of the casting and thereby the formation of the structure by grading the coefficient of heat transmission or the conductivity of the material used for the mold, in such a way

25 as to improve the quality of the casting. The invention consists in mixing into the substance used for the mold, a material the thermal conductivity of which in the unheated state is lower than that of iron but greater than that of sand,

30 and which is also highly refractory. Preferably the material, used by itself or as an admixture to others, will have in the unheated state a thermal conductivity lower than that of iron, but increasing with increasing temperatures until it is above

35 that of iron. A suitable material to use for regulating the thermal conductivity or heat transmission of the substance used for the mold is graphite.

40 The invention is based on adopting for the mold a material which, as compared with materials hitherto used for this purpose, possesses a very variable thermal conductivity. The coefficient of heat transmitted  $\lambda_1$  for a certain cast iron is for example 0.15 cal./sq. cm./second/degree C., the coefficient  $\lambda_2$  for a typical foundry sand is 0.0006.

45 The thermal conductivity of the new substance for

making molds can now, not only fill out by steps the interval at present existing between the thermal conductivity of the usual material and the thermal conductivity of iron, but it can also become greater than the thermal conductivity of iron.

According to the invention, graphite is preferably used as the material, or as a constituent of the mixed materials, for making the molds. The coefficient of heat transmission of graphite in the solid state is 0.105 cal./cm./second/degree C. when unheated, and 0.28 at a temperature of 555° C. (according to Landolt-Börnstein, Physikalisch-chemische Tabellen, 5th edition and supplementary volume, 1927).

If the coefficient of heat transmission of the usual foundry sand is taken as 1, the coefficient of heat transmission for cast iron is then about 250, and of the new molding substance using solid graphite, about 180 when unheated and about 470 at a temperature of 555° C.

Whilst the conductivity of the cast iron used for molds is 250 times greater than that of the usual foundry sand, and consequently also, when both substances are used simultaneously beside each other, the transmission of heat at a certain spot is 250 times greater than that at a neighboring spot, i. e. it suddenly changes; but on the other hand the conductivity of the new material for making molds changes gradually or by steps until it is 470 times greater than the conductivity of the usual foundry sand, the figure depending on whether it is unmixed, in the form of powder, in solid form or at a high temperature; consequently the thermal conductivity can be changed as required within the limits met with in practice.

By altering the proportions of the materials used for making molds, the coefficient of heat transmission can be gradually, and not only suddenly, changed, thereby increasing the qualities of the casting, without any drawbacks for the machining or for any other later process having to be put up with.

I claim:

1. A mold for casting metals comprising molding sand and a material, which in an unheated state, has a coefficient of thermal conductivity lower than that of iron and greater than that of the molding sand, said material being non-uniformly distributed throughout the molding sand and being present in greater proportion at those places where heat is to be removed more rapidly.
2. A mold for casting metals comprising molding sand and a material which, in an unheated state, has a coefficient of thermal conductivity

- lower than that of iron and greater than that of the molding sand, and which, when heated to casting temperatures, has a coefficient of thermal conductivity greater than that of iron, said material being non-uniformly distributed throughout the molding sand and being present in greater proportion at those places where heat is to be removed more rapidly. 80
5. A mold for casting metals comprising molding sand, and graphite non-uniformly distributed throughout the molding sand and being present in greater proportion at those places where heat is to be removed more rapidly. 85
3. A mold for casting metals comprising molding sand, and graphite non-uniformly distributed throughout the molding sand and being present in greater proportion at those places where heat is to be removed more rapidly. 90
4. A mold for casting metals comprising molding sand and a material which, in an unheated state, has a coefficient of thermal conductivity lower than that of iron and greater than that of molding sand, said material being non-uniformly distributed throughout the molding sand, the molding sand being free from inclusion of said material at places where the cast object has the least wall thickness, and the material being present in progressively increasing amounts to places where the cast object has the greatest wall thickness, so that the conductivity and the cooling rate at different places of the cast object are in accordance with the heat to be removed at those places for the purpose of improving the structure of the casting. 95
15. A mold for casting metals comprising molding sand and a material which, in an unheated state, has a coefficient of thermal conductivity lower than that of iron and greater than that of molding sand, said material being non-uniformly distributed throughout the molding sand, the molding sand being free from inclusion of said material at places where the cast object has the least wall thickness, and the material being present in progressively increasing amounts to places where the cast object has the greatest wall thickness, so that the conductivity and the cooling rate at different places of the cast object are in accordance with the heat to be removed at those places for the purpose of improving the structure of the casting. 100
20. A mold for casting metals comprising molding sand and a material which, in an unheated state, has a coefficient of thermal conductivity lower than that of iron and greater than that of molding sand, said material being non-uniformly distributed throughout the molding sand, the molding sand being free from inclusion of said material at places where the cast object has the least wall thickness, and the material being present in progressively increasing amounts to places where the cast object has the greatest wall thickness, so that the conductivity and the cooling rate at different places of the cast object are in accordance with the heat to be removed at those places for the purpose of improving the structure of the casting. 105
25. A mold for casting metals comprising molding sand and a material which, in an unheated state, has a coefficient of thermal conductivity lower than that of iron and greater than that of molding sand, said material being non-uniformly distributed throughout the molding sand, the molding sand being free from inclusion of said material at places where the cast object has the least wall thickness, and the material being present in progressively increasing amounts to places where the cast object has the greatest wall thickness, so that the conductivity and the cooling rate at different places of the cast object are in accordance with the heat to be removed at those places for the purpose of improving the structure of the casting. 110
30. 5. A molding for cast metals comprising mold-

MAX HEUSSER. 105

|    |     |
|----|-----|
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |